

## UNITED STATES PATENT OFFICE

2,123,261

## TEXTILE YARN

Matthew Michael Taylor and Stephen Miller Fulton, Spondon, near Derby, England, assignors to Celanese Corporation of America, a corporation of Delaware

No Drawing. Application December 22, 1936, Serial No. 117,146. In Great Britain February 5, 1932

15 Claims. (Cl. 117—52)

This application relates to composite yarns containing yarn having a basis of continuous filaments but having the appearance of spun yarn, i. e. of yarn made from staple fibre, and fabrics made therefrom. The application is in part a continuation of our co-pending application S. No. 746,258 filed 29th September, 1934, now Patent No. 2,077,441, which is in part a continuation of our application S. No. 712,120 filed 20th February, 10 1934, itself a continuation-in-part of our application S. No. 652,780, filed 21st January, 1933, now Patent No. 1,959,142 issued 15th May, 1934.

According to the invention yarns are made by twisting or doubling a plurality of individual 15 strands or yarns at least one of which is composed of short lengths of fibrous material and at least one other of which is an imitation spun yarn or stabilized yarn, and the invention includes fabrics made from these mixed yarns.

Throughout the specification and claims the term "regular yarn" is used to mean yarn formed by associating a plurality of substantially continuous filaments, and the term "spun yarn" is used to mean yarn formed by spinning relatively short lengths of filaments or fibres. The 25 stabilized yarn employed in making yarns according to the invention is formed by any suitable method from regular yarns by cutting, breaking or tearing operations so carried out that at any point in its length one or more of the filaments in the bundle of filaments constituting the 30 yarn are severed and one or more of the filaments in the bundle remain unsevered and the continuity of the bundle as a whole is not affected.

For example the methods described in U. S. Patents Nos. 1,956,600, 1,959,142, 2,031,647, 2,044,130 and 2,046,615 may be employed or the stabilized 35 yarns may be formed by the methods described in U. S. Patents Nos. 2,098,980, 2,096,795, 2,098,40 981 and 2,077,283.

The stabilized yarn may be formed from any desired regular yarn, for example, yarn of cellulose acetate or other organic derivative of cellulose, e. g. other cellulose esters such as cellulose 45 formate, propionate and butyrate and cellulose ethers such as methyl cellulose, ethyl cellulose and benzyl cellulose; yarn of wholly or partially and uniformly or intermittently saponified organic esters of cellulose; yarn of regenerated or 50 constituted cellulose such as viscose, nitrocellulose or cuprammonium artificial silk; natural silk yarns; and yarns consisting of a mixture of any two or more of these types, according to the effect desired in the mixed yarn. The stabilized yarn 55 may be, for example, lustrous, weighted and/or

pigmented. The number of filaments employed in the formation of the stabilized yarn may be from 10-200 or more and the denier of the yarns may be, for example, from 75-300 with any desired degree of twist from 3-20 or more turns per 6 inch.

The spun yarns may be formed by any suitable method of spinning staple length fibres, e. g. by the worsted method, the woollen method, the French method or the cotton method. Fibres 10 which constitute these yarns may be, for example, cotton or wool fibres, or artificial fibres, e. g. cellulose acetate staple fibre, and preferably are wool fibres having a staple length between 2 and 8 inches of a grade between 54's and 72's. 15 If desired staple length fibres of cellulose acetate or other organic derivatives of cellulose may be mixed with wool or cotton to form the spun yarn. The spun yarns may be of any suitable size and of any desired degree of twist, although it is generally preferable to employ spun yarns having a 20 count of 20-60 with a twist of 11-20 turns per inch.

With the stabilized and spun yarns there may be associated regular yarns, which may, for example, be formed by associating from 3 or 10 to 100 or 200 or more continuous filaments of the nature of those used in the regular yarns described above in connection with the formation of the stabilized yarns. The constituent 30 filaments of these regular yarns may be associated with substantially no twist or with a twist of up to 50 or more turns per inch.

The composite yarn may be formed by twisting or doubling together stabilized yarns and spun 35 yarns in any desired ratio; for example, one spun yarn may be twisted with one stabilized yarn or with 2, 3, 4 or more stabilized yarns.

The composite yarns may be formed from the several constituent yarns by twisting to an extent of, for example, 3-15 turns per inch. The twist imparted in the twisting or doubling operation may be in the same direction or in the opposite direction to the twist of the yarns forming the individual components. Furthermore, spun 45 yarn having a right-hand twist may be doubled with stabilized yarn having a left-hand twist, the two components being twisted together with either a left or right-hand twist.

The composite yarns made as described above 50 may be woven, knitted, knotted or netted into fabrics. These fabrics are wool-like in appearance and possess characteristics which render them particularly well suited for men's summer and winter suits and for women's light and heavy- 55

weight coats and suits; the fabrics are stronger than fabrics of similar appearance previously produced.

Attractive fabrics may be woven from the composite yarns of the invention, for example, in plain 1:1 weave or in patterns, herring bones, basket weaves and the like. The fabric may contain any desired number of warp ends or picks. Thus, for example, fabric may be woven in a 10 plain 1:1 weave having from 35-45 warp ends and from 30-45 picks.

After formation the fabric may be finished and dyed in the usual manner. It is found, moreover, that fabrics containing the composite yarns 15 of the invention are exceptionally well suited to napping operations by brushing the surface of the formed fabric. The fabrics are also noteworthy for their good draping powers, especially when containing regular yarns of organic derivatives of cellulose in addition to the spun yarns and stabilized yarns of organic derivatives of cellulose.

The following example illustrates the invention but is not to be regarded as limiting it in 25 any way:—

*Example*

A composite yarn is formed by twisting together with 8 turns right-hand twist, 3 ends of a 170 denier pigmented stabilized yarn having a 30 twist of 5 turns right-hand, and a spun worsted woolen yarn having a count of 40 and a twist of 14 right-hand turns per inch. The resulting composite yarn is woven into a fabric with a plain 1:1 weave having 42 warp ends and 34 35 picks.

Having described our invention, what we desire to secure by Letters Patent is:—

1. A composite yarn containing at least one spun yarn and at least one stabilized yarn.
2. A composite yarn containing at least one spun yarn of wool fibres and at least one stabilized yarn containing an organic derivative of cellulose.
3. A composite yarn containing at least one spun yarn of wool fibres and at least one stabilized yarn containing cellulose acetate.
4. A composite yarn containing at least one spun yarn of wool fibres of 18-60 count and having a twist of 11-20 turns per inch, and at least one stabilized yarn containing an organic derivative of cellulose.
5. A composite yarn containing at least one spun yarn of wool fibres of 18-60 count and having a twist of 11-20 turns per inch, and at least one stabilized yarn containing an organic derivative of cellulose and of denier between 75 and 200 with a twist of 3-20 turns per inch.

6. A composite yarn containing at least one spun yarn of wool fibres of 18-60 count and having a twist of 11-20 turns per inch, and at least one stabilized yarn containing an organic derivative of cellulose and of denier between 75 and 200 5 with a twist of 3-20 turns per inch, the constituent yarns being twisted together at 3-15 turns per inch.

7. A composite yarn containing at least one spun yarn of wool fibres of 18-60 count and having a twist of 11-20 turns per inch, and at least one stabilized yarn containing an organic derivative of cellulose and of denier between 75 and 200 10 with a twist of 3-20 turns per inch in the same direction as the twist of the spun yarn. 15

8. A composite yarn containing at least one spun yarn of wool fibres of 18-60 count and having a twist of 11-20 turns per inch, and at least one stabilized yarn containing an organic derivative of cellulose and of denier between 75 and 200 20 with a twist of 3-20 turns per inch in the same direction as the twist of the spun yarn, the constituent yarns being twisted together at 3-15 turns per inch in the same direction as the spun 25 yarn.

9. A composite yarn containing at least one spun yarn of wool fibres and at least three stabilized yarns containing an organic derivative of cellulose.

10. A composite yarn containing at least one 30 spun yarn of wool fibres of 18-60 count and having a twist of 11-20 turns per inch, and at least three stabilized yarns containing an organic derivative of cellulose and of denier between 75 and 200 with a twist of 3-20 turns per inch in the 35 same direction as the twist of the spun yarn.

11. A composite yarn containing at least one spun yarn, at least one stabilized yarn, and at least one regular yarn.

12. A composite yarn containing at least one 40 spun yarn of wool fibres, at least one stabilized yarn containing an organic derivative of cellulose, and at least one regular yarn containing an organic derivative of cellulose.

13. A fabric containing a composite yarn, said 45 composite yarn containing at least one spun yarn and at least one stabilized yarn.

14. A fabric containing a composite yarn, said composite yarn containing at least one spun yarn of wool fibres and at least one stabilized yarn 50 containing an organic derivative of cellulose.

15. A fabric containing a composite yarn, said composite yarn containing at least one spun yarn, at least one stabilized yarn, and at least one regular yarn.

MATTHEW MICHAEL TAYLOR.  
STEPHEN MILLER FULTON.